

## UNITED STATES PATENT OFFICE.

GILBERT C. BACON, OF STAMFORD, CONNECTICUT, ASSIGNOR TO ATLAS POWDER COMPANY, OF WILMINGTON, DELAWARE, A CORPORATION OF DELAWARE.

## PYROXYLIN-COATED FABRIC.

No Drawing.

Application filed January 3, 1925. Serial No. 449.

*To all whom it may concern:*

Be it known that GILBERT C. BACON, citizen of the United States, residing at Stamford, in the county of Fairfield and State of Connecticut, has invented certain new and useful Improvements in Pyroxylin-Coated Fabrics, of which the following is a specification.

This invention relates to the process of 10 coating a decorative fabric with a thin pyroxylin solution. It relates more particularly to that type of coated, or decorative fabrics described in United States Patent No. 1,450,367. Coated fabrics of this 15 type are formed by using a figured fabric, as cretonne, for example, though any suitable fabric may be employed, and applying a thin coating of pyroxylin, which, after drying, may be embossed or otherwise finished. In the manufacture of material of 20 the character mentioned, the desire is to produce an article that will be unaffected by light, will retain its original color, and will produce no harmful effect upon the pyroxylin coating. I have discovered that by using 25 a dye or dyes, of that class of dyes, known as indanthrene series, in the preparation of the fabric to be coated with a thin pyroxylin solution, it will not be affected by light, or 30 fade or discolor or otherwise injuriously affect the pyroxylin coating as is the case with some of the commonly used dyes.

Having thus described my invention, what 35 I claim as new and desire to secure by Letters Patent is:

1. A figured fabric which has been printed or dyed with that class of dyes known as the indanthrene series, having a thin coating of pyroxylin material.
2. A figured fabric which has been printed or dyed with that class of dyes known as the indanthrene series, having a thin coat-

ing of transparent pyroxylin, the surface of which, is embossed with a fine pebble grain.

3. A fabric which has been printed or 45 dyed with that class of dyes known as the indanthrene series, having a design imprinted thereon, and having a coating of a thin, transparent pyroxylin composition.

4. A fabric which has been printed or 50 dyed with that class of dyes known as the indanthrene series, having a design imprinted thereon, and having a coating of a thin, transparent pyroxylin composition, the surface of which, is embossed, to render it 55 irregular and thereby eliminate gloss so that the pattern of the design will be visible at all angles, through the said coating.

5. A fabric which has been dyed with that 60 class of dyes known as the indanthrene series, said fabric having a thin coating of pyroxylin material.

6. A fabric which has been printed or 65 dyed with that class of dyes known as the indanthrene series, having a design printed thereon, and a thin coating of transparent or semi-transparent pyroxylin, the surface of which is embossed with a design corresponding to the figures printed on the fabric.

7. A fabric which has been printed or 70 dyed with that class of dyes known as the indanthrene series, having a design imprinted thereon, and having a thin coating of a transparent pyroxylin composition, the surface of which is embossed with a fine pebble grain.

In testimony whereof he affixes his signature in the presence of two witnesses.

GILBERT C. BACON.

Witnesses:

W. N. STOCKTON,  
H. E. SAUENGER,